

## UNITED STATES PATENT OFFICE

2,347,916

CONTAINER CONTAINING HYDROGEN  
SULPHIDE VAPOR

Clifford P. Larrabee, Vandergrift, Pa.

No Drawing. Application December 3, 1942,  
Serial No. 467,785

5 Claims. (Cl. 206—84)

This invention relates to steel containers containing hydrogen sulphide vapor, the object being to provide an inexpensive steel container capable of resisting the peculiar corrosion properties of this vapor. Such a steel container is exemplified by a steel storage tank containing sour petroleum oil which includes sulphur compounds and fills the tank inside, unoccupied by the oil itself, with vapor consisting of hydrogen sulphide, moisture and air.

Since cost prohibits the use of high-alloy steels, exemplified by the stainless steels, which adequately resist corrosion of this vapor, such steel containers are conventionally made of plain-carbon or low-alloy structural steel. Heretofore, it has not been known how to make such steel adequately resistant to the corrosion of hydrogen sulphide vapor, the storage tank mentioned having an undesirably short service life due to corrosion of its parts contacted by the vapor.

The present invention is predicated on the discovery that, with but one exception, any of the plain-carbon or low-alloy structural steels may have its resistance to corrosion by hydrogen sulphide vapor, greatly increased by the addition of relatively small amounts of arsenic, which do not materially affect its cost. The exception is represented by those steels containing both chromium and nickel with both these elements in excess of .25%. However, when either of these elements exceeds .25%, it can be rendered harmless, to the described effect of the arsenic, by keeping the other of these elements below .25%. Because of cost, neither chromium nor nickel should be included in excess of the percentages within low-alloy ranges, this, generally speaking, limiting these elements to 5% maximums. Otherwise, the use of arsenic seems to function properly to increase the corrosion resistance to the vapor, in the case of any of the steels mentioned as conventionally used where cost excludes the high-alloy types.

It follows that the invention consists of a steel container containing hydrogen sulphide vapor made of steel containing an amount of arsenic effecting an increase in its resistance to corrosion by this vapor and with its balance iron excepting for elements harmless to this effect of the arsenic.

More specifically, the arsenic should preferably range in content from .05 to 1.50%, and the maximum increase in resistance to corrosion by this vapor is effected by about a 1% arsenic content. If the steel includes chromium and nickel, the contents of these elements must be adjusted so that when one is present in excess of .25%, the

other is present in a lower percentage, neither of these named elements being present in sufficient amount, in any event, to provide the effect of the arsenic to the same degree. In other words, there is no point in using the arsenic to effect a low-cost product of increased corrosion resistance, when the steel is of the high-alloy chromium or chromium-nickel type. Furthermore, there is no point in increasing either expensive element to a point where, by itself, the steel's resistance to the vapor is increased beyond what could be afforded by the arsenic.

Since the arsenic works with any of the structural steels, the invention may be defined as a container containing hydrogen sulphide vapor, made of steel containing from .05 to 1.05% carbon, from .25 to 1.20% manganese, a maximum of .055% sulphur, a maximum of .20% phosphorus, from .50 to 1.50% arsenic, effecting an increase in its resistance to corrosion by the vapor, and the balance mainly iron. These compositional ranges cover the structural steels generally. In the case of the low-alloy structural steels, the balance is still considered as being mainly iron, this term being construed herein as covering the alloy amounts which are used in this type of steel. Therefore, the steel may contain from smaller amounts to not more than 5% of chromium or 5% of nickel, with the contents of these two just-named elements adjusted, if used together, so that the content of one is less than .25% when the other exceeds this amount. Actually, these two elements are not normally used in such maximum amounts because of cost, but are usually restricted to a value less than 3%.

Heretofore, it has been known that arsenic, along with copper, phosphorus, chromium, nickel, etc., enhance the resistance of the low-alloy structural steels to corrosion of other types. But it has not been known that of all these various alloys, arsenic exerts a critically greater increase in the resistance of such steels to corrosion by hydrogen sulphide vapor, than do equal amounts of any of the others. The most practical embodiment of the arsenic, is to include it as the sole alloy in what would otherwise be a plain-carbon structural steel, but other alloys may be required to meet special physical requirements.

It is to be understood that the phosphorus content must be adjusted respecting the carbon content. In general, when the carbon content does not exceed about .10%, 1.20% phosphorus may be used, while with carbon contents exceed-

ing about .20%, the phosphorus content should not exceed about .045%.

I claim:

1. A container containing hydrogen sulphide vapor, made of steel containing from .05 to 1.50% arsenic effecting an increase in its resistance to corrosion by this vapor and with its balance iron excepting for elements harmless to this effect of the arsenic.

2. A container containing hydrogen sulphide vapor, made of steel containing about 1% arsenic effecting an increase in its resistance to corrosion by this vapor and with its balance iron excepting for elements harmless to this effect of the arsenic.

3. A container containing hydrogen sulphide vapor, made of steel containing from .05% to 1.50% arsenic effecting an increase in its resistance to corrosion by this vapor and with its balance iron excepting for elements harmless to this effect of the arsenic, including chromium and nickel with the contents of these elements adjusted so that when one is present in excess of .25% the other is present in a lower percent-

age, neither of these named elements being present in sufficient amount to provide the effect of the arsenic to the same degree.

4. A container containing hydrogen sulphide vapor, made of steel containing from .05 to 1.05% carbon, from .25 to 1.20% manganese, a maximum of .055% sulphur, a maximum of .12% phosphorus, from .50 to 1.50% arsenic effecting an increase in its resistance to corrosion by the vapor, and the balance mainly iron.

5. A container containing hydrogen sulphide vapor, made of steel containing from .05 to 1.05% carbon, from .25 to 1.20% manganese, a maximum of .055% sulphur, a maximum of .12% phosphorus, from .50 to 1.50% arsenic effecting an increase in its resistance to corrosion by the vapor, and the balance mainly iron, including from smaller amounts to not more than 5% of chromium and 5% nickel with the contents of these last two named elements adjusted so that the content of one is less than .25% when the other exceeds this amount.

CLIFFORD P. LARRABEE.